

## UNITED STATES PATENT OFFICE

HARRY K. HERSCHEMAN, OF WASHINGTON, DISTRICT OF COLUMBIA, AND JOHN L. BASIL,  
OF ANNAPOLIS, MARYLAND

## METAL ALLOY

No Drawing.

Application filed August 17, 1932. Serial No. 629,392.

(GRANTED UNDER THE ACT OF MARCH 3, 1883, AS AMENDED APRIL 30, 1928; 370 O. G. 757)

The invention described herein, if patented, may be manufactured and used by or for the Government for governmental purposes without payment of any royalty 5 thereon.

This invention relates to improvements in metal alloys and more particularly to a copper base alloy of high lead content especially adapted for use in bearings, it being understood 10 that numerous other uses will be found for such an alloy.

An object of this invention is to provide a bearing metal of especially low frictional properties and having the following additional properties combined: high melting point, high strength, toughness, high wear resistance and proper hardness and conformability, and further, especially improved properties at elevated temperatures.

20 A further object in view is to provide all of the above without the use of tin, which is not only an expensive but a strategic metal obtainable only in small quantities in this country.

25 The present type of copper base bearing metals with particular reference to those containing lead, have lead 10-28 percent; tin 2-10 percent, and the remainder copper and minor impurities. The above is commonly known to the trade as lead bronze bearing metal and is the type of bearing metal improved by the discovery herein disclosed.

30 A satisfactory bearing metal should for obvious reasons be so composed as to tend 35 to prevent seizure between the bearing and the shaft, when lubrication may for any reason fail. To provide such a bearing metal, alloys containing large percentages of lead or other metals of the same characteristics are used.

Bearing metals subjected to heavy loads and high speeds cannot be made entirely of lead due to the fact that it does not have sufficient load-carrying ability. In order to 45 give lead sufficient support for such service other metals are combined with it. In such combinations copper is usually used and forms a matrix in which the lead is distributed. In order to properly distribute the lead

uniformly as discontinuous particles through the matrix, other elements are added.

The matrix which is the strengthening and stiffening element should provide continuous envelopes of copper or of the solid solution 55 of these elements in copper, thus distributing the lead in globular and discontinuous form throughout the mass.

Copper and lead are known to be miscible and will alloy in nearly all proportions when 60 heated to sufficiently high temperatures. They, however, separate out when cooled since these metals remain alloyed to a very negligible degree when cooled to room temperatures. In the prior art certain elements 65 such as tin and sulphur have been added to prevent such separation. The degree of success with which this has been accomplished by the addition of these elements has been limited and the bearing metals so produced 70 have failed to meet all the requirements which are known to be essential to an efficient and successful bearing for operation at high speeds and high pressures with the result that they are unsuitable or deficient in one or all 75 of the properties above referred to.

Further, in order that a bronze bearing metal meet all of the above requirements for the property of conformability, it is necessary that the matrix of the bearing metal be 80 sufficiently soft and the lead content sufficiently high, to allow for the so-called "wiping action" and flow of the bearing to prevent seizure, which should be accomplished without sacrificing the necessary strength, toughness, and wear resistance required at high operating temperatures resulting from increasingly high speeds and high powers being developed in internal combustion motors and similar fields.

The subject matter of this invention, which 90 fully meets the conditions wherein a highly satisfactory bearing metal is provided without the use of tin, consists of lead up to about 40 percent, sulphur about 0.2 to 0.6 percent, 95 silicon about 0.2 to 1.0 percent, zirconium about 0.3 to 1.5 percent, and copper, the balance. The silicon and zirconium may be obtained as a commercial alloy containing silicon 35-39 percent, zirconium 50-55 percent, 100

and small amounts of other elements. The silicon-zirconium alloy may be prepared with other variations of silicon and zirconium than those referred to. Desired results may be obtained by higher or lower percentages of the elements mentioned, it having been found that alloys containing additions of various amounts of sulphur, silicon, and zirconium permit the use of relatively high percentages of lead showing same to be present in the matrix in well distributed, fine and discontinuous particles.

While it is known that the addition of sulphur alone will permit the use of high lead content with good distribution, the lead in such instances is present in the form of continuous envelopes around the grains of copper. Under such conditions the metal does not have the strength of one in which the lead particles are discontinuous and well distributed in the matrix. The addition of silicon and zirconium together with sulphur, has very definitely been found to break up the envelope formation of lead and provide finely divided globular particles of lead filling the interstices in the unbroken network of the copper base matrix. The silicon and zirconium either separately or together, further give improved mechanical properties to the bearing metal at elevated temperatures.

The improved alloy here described not only permits a higher percentage of lead content than possible in the former art but also shows no appreciable effect in its composition or structure when remelted and cast a plurality of times.

The method of preparing this improved bearing metal is as follows: Melt down the copper in any suitable furnace, add the lead thereto when the copper is molten, then add the silicon-zirconium alloy which has preferably first been made up as a "hardener" containing copper 90 percent, silicon-zirconium alloy 10 percent, after all of the metals while molten, have been thoroughly mixed, sulphur is added in the form of elemental sulphur or as lead or copper sulphide.

It will be understood that variations may be practiced in the preparation of the improved bearing metal as follows: Melt down the copper, add the lead thereto when the copper is molten, then add silicon which has preferably been first prepared as a "hardener" containing copper 90 percent, silicon 10 percent, then add zirconium which has preferably first been made up as a "hardener" containing copper 90 percent, zirconium 10 percent, after all the metals while molten have been thoroughly mixed, sulphur is added.

The above sequence may be varied, for instance, the silicon and zirconium prepared as "hardeners" may be added to the molten copper, prior to adding the lead. The molten mass after all additions have been made,

should be heated to a sufficiently high temperature to insure thorough alloying of all the elements present.

A preferred method of preparing this alloy with special reference to temperatures, is to heat the copper to approximately 1100-1200 degrees C., add the lead to the molten copper, then add the silicon and zirconium to the molten metal which is maintained at about 1150-1200 degrees C. to insure complete alloying of the constituents, cool the melt to about 1125 degrees C. and add sulphur, following which the molten mass may be cast.

It will be understood that silicon-zirconium need not be added in the forms above described, but may be added, as alloys of iron-silicon, manganese-silicon, iron-zirconium and other similar alloys, with wholly beneficial effects though not to such an extent as in the form described.

Having thus fully described our invention what we claim and desire to secure by Letters Patent is:

1. An alloy composed of, about 60 percent by weight of copper, about 38 percent by weight of lead, about 1.5 percent by weight of silicon-zirconium alloy and about 0.4 percent by weight of sulphur.

2. A bearing alloy comprising, about 60 percent by weight of copper, about 38 percent by weight of lead, about 1.5 percent by weight of silicon-zirconium alloy adapted to distribute the lead and harden and strengthen the bearing alloy and about 0.4 percent by weight of sulphur adapted to distribute the lead.

3. An alloy composed of, copper about 60 percent by weight, lead about 38 percent by weight, silicon zirconium alloy 0.5 to 2.5 percent and 0.2 to 0.6 percent sulphur in the form of copper sulphide.

4. An alloy composed of, copper about 60 percent by weight, lead about 38 percent by weight, silicon zirconium alloy 0.5 to 2.5 percent and 0.2 to 0.6 percent of sulphur in the form of lead sulphide.

5. An alloy consisting of copper, lead, silicon, zirconium and sulphur in which the sulphur represents about 0.4 percent by weight, silicon about 0.6 percent, zirconium about 0.9 percent, the copper about 60 percent, and the lead constituting the remainder.

6. An alloy consisting of copper, lead, silicon, zirconium, and sulphur which represents sulphur 0.2 to 0.6 percent by weight, silicon 0.2 to 1.0 percent, zirconium 0.3 to 1.5 percent, the lead in substantial amounts up to 40 percent and copper the balance.

HARRY K. HERSCHEMAN.  
JOHN L. BASIL.